

## UNITED STATES PATENT OFFICE

2,053,853

LOW POUR POINT MINERAL OIL  
COMPOSITION

Adrianus Johannes van Peski, Bussum, Netherlands, assignor to Shell Development Company, San Francisco, Calif., a corporation of Delaware

No Drawing. Application July 1, 1933, Serial No. 678,716. In the Netherlands July 5, 1932

6 Claims. (Cl. 87—9)

This invention relates to the methods of lowering pour points of mineral oils, and is particularly concerned with the class of viscous lubricating oils containing waxy constituents.

5 The invention resides in the discovery that certain organic compounds upon being added to mineral oils in very minute quantities markedly lower the pour points of these mineral oils. The effect of adding such substances to mineral oils 10 may be determined by various methods, such, for example, as A. S. T. M. Method D 97—27T.

According to this invention the active organic substances to be used for lowering the pour points of mineral oils, i. e. the substances possessing 15 pour point reducing properties, are built up of cyclic nuclei and aliphatic side chains, the latter containing at least one oxygen or nitrogen atom, preferably in such a way that if the substance contains only one nucleus at least two side chains 20 are present and if the substance contains more than one nucleus at least one side chain is present. These products are for example obtained as reaction products of the fatty acids and/or alcohols with cyclic compounds whose molecules contain 25 two or more primary amino, and/or one or more secondary-amino and/or hydroxy, and/or poly-hydroxy, and/or amino-hydroxy groupings. The mono- or poly-cyclic nuclei to which one or more radicles of a fatty acid and/or an 30 alcohol are attached may be either heterocyclic or carbocyclic. The nitrogen atom or atoms connecting the cyclic nucleus with the fatty acid radicles may be either within the nucleus as in azines or oxazines, or attached directly to a carbon atom of the nucleus.

Among various nitrogen-containing compounds the secondary mono- or poly-amines and particularly the primary poly-amines were found to be suitable for producing in combination with the 40 higher fatty acids (or better, with their anhydrides, or corresponding acyl-halides) the pour point reducing substances. For example, among such suitable compounds may be mentioned: o-, or m-, or p-phenylene-diamines, or triamino-, or 45 tetramino-benzenes, also their homologues with one or more alkyl side chains, such as diamino-toluenes, diamino-methylethyl-benzene, diamino-xylenes, triamino-toluenes, triamino-ethyl benzenes, triamino-xylenes, triamino-azo-benzene 50 hydrochloride (Bismarck brown), etc. Representing the secondary monoamino- and secondary poly-amino-aryl compounds may be mentioned: diphenylamine, methylaniline, and their homologues, methyl aminoaniline, dimethylphenylene-diamine, phenylaniline-amine - methylphenyl -

phenylene-diamine, and their homologues. The group —NH—, as has been stated, may be positioned within the nucleus of the molecule, as for example in benzopyrrole, or indole, or in indigo.

It is to be understood that tertiary amines may be used for the purpose of this invention, provided, however, that they contain a primary and/or secondary amino groupings in addition to the tertiary one.

The above enumerated groups of nitrogen-containing compounds, and particularly such compounds as 1,3,phenylene diamine, indigo, and Bismarck brown, were found to produce, when allowed to react in conventional manner with fatty acids, or their anhydrides, or corresponding acyl halides, substances possessing properties of lowering the pour points of mineral oils containing waxy constituents. Such reaction products are known to be amides of the acids used in the reactions, such as anilides.

Referring now to the oxygen-containing groups of the compounds suitable for the purpose of the present invention, these were stated to include hydroxy-, polyhydroxy-, and amino-hydroxy-cyclic compounds, which may be represented by such specific examples from aromatic series as: phenol, di- and/or tri-hydroxy benzenes and their homologues, mono-, or di-, or tri-hydroxy naphthalenes, or mono-, and/or poly-hydroxy-anthra- 30 cenes, or mono-, or poly-hydroxy-anthraquinones, and their homologues; also compounds of the aurine group, such as aurine (a trihydroxy-triphenyl-methane), compounds of hydroxy-amino-benzene and hydroxy-polyamino-benzene groups, etc.

In order to obtain the desired pour point reducing substances, the oxygen containing compounds are made to react in a known manner with the higher fatty acids (or their anhydrides, or acyl halides), such as stearic, palmitic, or cerotic acids, and/or with one or more of the lower and/or higher aliphatic primary, secondary or tertiary alcohols, which may be either mono-, or poly-hydroxy, and either saturated or unsaturated. The resulting products of reaction may be either 45 ketones or ethers or esters, or amido-salts of the fatty acids used in the reaction, or mixed ethers or esters and amido-salts.

It should be noted that this invention is not dependent upon or limited to the particular methods of obtaining the substances possessing pour point reducing properties, but is directed to the use of such substances regardless of the methods of their manufacture. In other words, even though these substances are defined in this speci- 55

5 fication as the reaction products of certain compounds, and/or groups of compounds, the same substances can be reproduced by other known methods and from other sources which may be different from those herein described, and such substances are to be understood to be within the scope of this invention.

10 For the purpose of illustrating more specifically the nature of the pour point reducing substances of this invention and their effect on a number of oils the following table has been made:

Oils

| 15 Pour point reducing substance            | Percent by wt. added | Lowering of pour points, ° C., from the original |                        |                         |
|---------------------------------------------|----------------------|--------------------------------------------------|------------------------|-------------------------|
|                                             |                      | Rumanian original p.p. +2° C.                    | Penn. org. p.p. -1° C. | Borneo org. p.p. +3° C. |
| 20                                          |                      |                                                  |                        |                         |
| 1. Distearyl m-phenylene diamine.           | .5                   | 23° C.                                           | -----                  | -----                   |
| 2. Stearyl compound of Bismarck brown.      | .5                   | -----                                            | -----                  | 8                       |
| 25 3. Stearyl compound of indigo.           | .5                   | 18                                               | 22                     | 14                      |
| 4. Tetrastearyl compound of triaminophenol. | .5                   | -----                                            | -----                  | 11                      |
| 5. Resorcinol-distearate.                   | .5                   | -----                                            | 5                      | -----                   |
| 6. Pyrogallol-tristearate.                  | .2                   | 20                                               | -----                  | -----                   |
| 7. Pyrogallol-tristearate.                  | .5                   | -----                                            | 9                      | -----                   |
| 8. Phloroglucinol-tristearate.              | .5                   | 20                                               | 5                      | -----                   |
| 30 9. Distearate of 1,5-dioxy-naphthalene.  | .1                   | 18                                               | -----                  | -----                   |
| 10. Aurine-distearate.                      | .5                   | -----                                            | 12                     | -----                   |
| 11. Trioxy-triphenylmethane-tristearate.    | .5                   | 20                                               | -----                  | -----                   |
| 12. Distearylalizarine.                     | 1                    | 15                                               | -----                  | -----                   |
| 35 13. Rufgallic acid-hexastearate.         | .5                   | 24                                               | -----                  | 17                      |

40 In addition to the above described groups of substances distearylnaphthalene the dimyricyl ether of 1,5-dioxy naphthalene and the cerotic acid ester of cholesterol were found very suitable for lowering pour points of mineral oils.

45 The products of reaction between a fatty acid, such as stearic acid, in the presence of  $AlCl_3$ , and the condensation products of naphthalene, such as described by Homer in the Journal of the Chemical Society of London, Transactions, 1907, vol. XCI, part II, page 1103, were found to be very effective pour point reducers, whose addition in quantities of about .5% by weight to the Rumanian, Pennsylvania, and Borneo oils lowered their respective pour points by 27° C., 25° C. and 9° C.

55 In general, the extent to which the pour point can be reduced by means of a particular substance depends upon the nature of the oil to be treated, so that some substances have a greater effect on one oil than on another. Some substances may have no effect on certain oils, but reduce the pour points of others. The most effective pour point reducer can be easily ascertained in each case by actual trials by using some of the various substances which have been described above. The optimum quantities of the selected pour point reducers may vary for different oils, but usually do not exceed 1% by weight of the oil.

60 It has been found that petroleum sulphonic

5 acids, i. e. those kinds thereof in which the sulphonate acid groups have entered into the aromatic nucleus of the molecule, can be converted into the corresponding phenols, by dissolution with potassium hydroxide and that compounds of the type according to this specification can be prepared therefrom by etherification or esterification with derivatives of high molecular alcohols or acids, which compounds can then be used as pour point reducers.

10 The compounds of the type described in this specification can be used not only to lower the pour points of natural and synthetic lubricating oils but can be used to lower the pour points of other hydrocarbon oils, for example, fuel oils, 15 gas oils, tar oils, shale oils and residues.

The compounds can advantageously be used in oil wells with a view to avoiding crystalline paraffin wax deposits.

20 I claim as my invention:

1. A mineral oil composition comprising a mineral oil and a small proportion of rufgallic acid hexastearate.

25 2. A mineral oil composition comprising a mineral oil containing waxy constituents in quantities sufficient normally to cause an undesirably high pour point and a small quantity of a compound having an organic cyclic nucleus and a side chain of the formula  $R-C(O)-O-R'$  where  $R$  represents a high-molecular organic radical containing said high molecular aliphatic chain and  $R'$  represents an organic cyclic nucleus, at least two radicals of the group consisting of ester, keto, ether and amido radicals being linked to  $R'$  when  $R'$  represents a single 35 monocyclic nucleus.

3. A mineral oil composition comprising a mineral oil containing waxy constituents in quantities sufficient normally to cause an undesirably high pour point and a small proportion of an ester 40 of a higher fatty acid and an organic cyclic compound, said ester containing at least two aliphatic side chains each linked to said cyclic compound through an ester group when said cyclic compound contains only one monocyclic 45 ring structure.

4. A mineral oil composition comprising a mineral oil containing waxy constituents in quantities sufficient normally to cause an undesirably high pour point and a small proportion of an ester 50 of a higher fatty acid and an organic carbocyclic compound, said ester containing at least two aliphatic side chains each linked to said cyclic compound through an ester group when said cyclic compound contains only one mono- 55 cyclic ring structure.

5. A mineral oil composition comprising a mineral oil containing waxy constituents in quantities sufficient normally to cause an undesirably high pour point and a small quantity of resorcinol distearate.

60 6. A mineral oil composition comprising a mineral oil containing waxy constituents in quantities sufficient normally to cause an undesirably high pour point and a small quantity of pyrogallol tristearate.

65 ADRIANUS JOHANNES VAN PESKI.